

A. PACZ.

PROCESS OF TREATING DRAWN METAL.

APPLICATION FILED APR. 13, 1914. RENEWED MAY 18, 1918.

1,280,825.

Patented Oct. 8, 1918.

FIG. 1.



FIG. 2.



WITNESSES:

Benjamin B. Clark  
Orlen Drford

INVENTOR:

ALADAR PACZ,  
BY Almon H. Davis  
His ATTORNEY.

# UNITED STATES PATENT OFFICE.

ALADAR PACZ, OF CLEVELAND, OHIO, ASSIGNOR TO GENERAL ELECTRIC COMPANY, A CORPORATION OF NEW YORK.

## PROCESS OF TREATING DRAWN METAL.

1,280,825.

Specification of Letters Patent.

Patented Oct. 8, 1918.

Application filed April 13, 1914, Serial No. 831,612. Renewed May 18, 1918. Serial No. 235,391.

To all whom it may concern:

Be it known that I, ALADAR PACZ, a citizen of the United States, residing at Cleveland, county of Cuyahoga, State of Ohio, 5 have invented certain new and useful Improvements in Processes of Treating Drawn Metal, of which the following is a specification.

My invention relates to the manufacture 10 of metal wire such as that used for making filaments and filament supports for incandescent lamps. More specifically, my invention comprises a process of treating during the drawing process, or immediately there- 15 after, wire such as that used for filaments and so as to render it better adapted for the work which it is called upon to perform.

My invention is particularly applicable to tungsten wire which is used for filaments 20 and filament supports in electric incandescent lamps. Drawn tungsten wire is produced according to the process described in Coolidge Patent No. 1,082,933, issued Dec. 30, 1913, and my invention is particularly 25 adapted to the treatment of wire which has been produced according to this process. As disclosed in the said Coolidge patent, the process of drawing down the wire comprises a number of steps, the wire being reheated a 30 number of times preparatory to passing through the various dies. My invention may be applied from time to time during the drawing down of the metal according to the said process, but I prefer to apply it after 35 the wire has been drawn down to approximately the final size for use as a filament or support in an incandescent lamp.

Tungsten wire produced prior to my invention, while very efficient and giving good 40 results in lamps, was rather difficult to mount upon the supports without a preliminary shaping, which required the heating of each filament. In order to keep the wire straight, the practice was to crimp it. More- 45 over, on account of the necessity of using a carbonaceous lubricant in drawing down wire a certain amount of carbon was physi- 50 cally or chemically included in the filament which naturally was of more or less disad- vantage in the lamps.

I have found that by giving the wire a preliminary heating at approximately red 55 heat in the presence of an oxidizing agent, preferably air or oxygen, the metal becomes inelastic and capable of taking a permanent

set without necessitating the preliminary shaping practised heretofore. After this first heating the wire is reheated in a non-oxidizing atmosphere to a much higher temperature, which may approach that to which 60 the metal will be exposed in an incandescent lamp. Preferably this atmosphere is reducing.

I do not wish to be confined to any particular theory as to what takes place during 65 the process constituting my invention. It is probable that the action which takes place is a combined chemical and physical one and includes the removal of impurities, such as carbon, and a change in the sizes of grains 70 due to rearrangement of molecules or ultimate particles of the metal. The wire which has been treated according to my invention is much superior to that heretofore produced in point of pliability and flexibility. It is 75 also much softer and takes a permanent set much more easily, remaining straight without requiring to be crimped.

In the drawing I have illustrated an apparatus by means of which one species of my 80 invention may be carried out. Figure 1 thereof is a sectional elevation of such an apparatus and Fig. 2 is a transverse section thereof on the line 2-2.

In applying the apparatus illustrated in 85 the drawing to the practice of my invention, the wire, which may be ductile tungsten produced by the process described in the Coolidge patent hereinbefore referred to, is placed upon the reel 10 and is led through 90 the apparatus to the reel 11 upon which it is wound by a suitable rotating mechanism 12. The tube 13, which is suitably supported by standards 14 is preferably cylindrical in shape and has a slot 15 formed in the top 95 thereof. At each end the said tube is provided with a mercury container 16 through which the wire passes and makes contact. A source of electric energy is connected by means of the leads 17 to the mercury contacts. 100

The tube 13 is open to the air on account of the slot in the top thereof and the air probably serves as an oxidizing medium to combine with the carbon and possibly other 105 impurities and their compounds contained in and on the wire which passes therethrough. The voltage between the contacts 16 is so regulated that the wire will be heated approximately to dull redness so that 110

the impurities will be attacked without seriously affecting the tungsten. The length of the tube 13 and the speed at which the wire travels therethrough are such as to allow time for the air to fully attack the impurities. I have found that if tube 13 is approximately one inch and a half in diameter and the distance between the contacts therein is approximately thirty-four inches, a speed of fifty feet per minute is suitable.

To the left of Fig. 1 is illustrated a second tube 18. This tube is closed at each end by the plugs 19, each of which supports a mercury contact 20 through which the wire passes. This tube is suitably supported by the members 21. The tube 18 is filled with a gas from which oxygen and other reagents which would attack the metal are absent. I prefer a reducing atmosphere and have used successfully forming gas composed of approximately 88 parts nitrogen and 12 parts hydrogen. This reduces any tungsten oxid formed during the previous treatment. The voltage between the contacts 20 is so regulated that the wire will be heated at least to a white heat.

In order that the wire may be observed during its passage through tube 18, this tube is preferably composed of glass or other transparent material, the length of the tube 18 must be such that the wire will not be subjected too long to the high heating. I have found that, when the first treatment is performed under the conditions heretofore stated, the distance between the contacts in tube 18 should be approximately seven inches.

According to one theory which I have evolved, in addition to having the physical effect hereinbefore referred to, the heating of the wire in the oxidizing atmosphere causes the carbon near the surface to burn and that which is contained within the wire to be sweated out to the surface. This sweating process may include the formation of a tungsten oxygen carbon compound. During the subsequent high heating of the wire in the absence of oxygen, any compounds which may have been formed by the oxygen are broken up and driven off.

During the second treatment the wire is shrunk and cleaned. The action which probably takes place is that the spaces formerly occupied by the carbon and other impurities are filled up with the pure metal, while any oxid which may have formed is removed by the hydrogen.

My process may be performed upon the wire at various stages of the drawing process. This has the advantage over treating the wire of the final size that the carbon or other impurity is not allowed to penetrate so far into the wire and its removal is therefore accomplished more easily.

The bent results have been achieved in

connection with tungsten wire produced from material which has been treated so as to obviate subsequent "offsetting" when used as a filament, for example, as described in the Coolidge patent hereinbefore referred to and in French Patent No. 1,089,757, March 10, 1914. However, good results have been secured with other wire.

What I claim as new and desire to secure by Letters Patent of the United States, is,—

1. The process of treating drawn metal which has been subjected to the action of impurities during its manufacture which consists in heating it at a comparatively low temperature while in contact with a re-agent which will combine with said impurities and afterward heating it to a comparatively high temperature in the absence of said re-agent.

2. The process of treating drawn tungsten which has been subjected to the action of impurities during its manufacture which consists in heating it at a comparatively low temperature while in contact with an oxidizing agent and afterward heating it to a comparatively high temperature in the absence of said oxidizing agent.

3. The process of treating drawn tungsten which has been subjected to the action of carbonaceous material during its manufacture which consists in heating it to a comparatively low temperature in the presence of a re-agent which will combine with carbon or carbon compounds and afterward heating it to a high temperature in the absence of such re-agent.

4. The process of treating drawn tungsten which has been subjected to the action of carbonaceous material during its manufacture which consists in heating it to a comparatively low temperature in the presence of an oxidizing agent and afterward heating it to a high temperature in the absence of such oxidizing agent.

5. The process of treating drawn tungsten which has been subjected to the action of carbonaceous material during its manufacture which consists in heating it to a comparatively low temperature in the presence of air and afterward heating it to a high temperature in an inert or reducing atmosphere.

6. The process of treating drawn tungsten which has been subjected to the action of carbonaceous material during its manufacture which consists in heating it to a low red heat in the presence of an oxidizing agent and afterward heating it approximately to a white heat in the absence of said oxidizing agent.

7. The process of treating drawn tungsten which has been subjected to the action of carbonaceous material during its manufacture which consists in heating it to a low red heat in the presence of an oxidizing agent

and afterward heating it approximately to a white heat in the presence of a reducing agent.

8. The process of treating drawn tungsten wire which consists in holding it at substantially red heat for a short period and afterward holding it at a white heat.

In witness whereof, I have hereunto set my hand this 26th day of March, 1914.

ALADAR PACZ.

Witnesses:

PAUL BACHMANN,  
JOHN I. OWENS.